

1

3,105,756

**METHOD OF LOWERING THE IRON CONTENT  
OF CHROMITE ORES OR CONCENTRATES  
WITHOUT APPRECIABLE LOWERING OF THE  
CONTAINED Cr<sub>2</sub>O<sub>3</sub>**

George E. Green, Baguio, Republic of the Philippines, assignor to Healmor Corporation, Dover, Del., a corporation of Delaware

No Drawing. Filed June 18, 1959, Ser. No. 821,091

3 Claims. (Cl. 75—1)

This invention relates to the mineral known as chromite, in any ores or concentrates, of any degree of fineness, that are termed "chromite" and that consist essentially of the oxides of chromium, iron, magnesium and aluminum in variable proportions, and has for its object an improved method for the extraction of part of the iron from the chromite mineral without appreciable lowering of the chromite content, thus in effect, raising the chromium:iron ratio to a higher factor than the ratio originally present.

The usual chemical formula used for chromite is FeO.Cr<sub>2</sub>O<sub>3</sub>, and pure chromite should theoretically contain 68% chromic oxide and 32% ferrous oxide. Pure chromite is not found in nature, since in all natural deposits part of the chromium and part of the iron has been replaced by aluminum and magnesium. For metallurgical grade chromite, a chromite material containing a minimum of about 45% Cr<sub>2</sub>O<sub>3</sub> is required, and a chromium:iron ratio of at least 3:1 is a requisite. Metallurgical grade chromite of this character is the type required for the fabrication of alloys of chromium. The most highly industrialized countries have no commercial deposits of this grade. There are many deposits in many countries, wherein the chromium:iron ratio is 2:1 or 2.5:1, and wherein the chromium content after mechanical concentration would be sufficiently high if a part of the iron could be removed without lowering the chromium content.

Work in the past, to the best of my knowledge, has been devoted chiefly to attempts to leach out part of the iron by very fine grinding followed by leaching under pressure, at high temperatures for long periods of time with strong, expensive solvents. The costs of treatment by such methods have precluded favorable economic results, and the loss of chromite invariably experienced has not only meant a further charge against such processes but has also partly nullified the improvement in the chromium:iron ratio otherwise resultant.

In my improved process for raising the chromium:iron ratio, I can make it possible to lower the iron to any economically desirable point without loss of more than 1% of the chromium content, using relatively small quantities of inexpensive reagents available everywhere, and since the iron leaching is done at air temperature, at atmospheric pressure, and in a few minutes time, the process can be continuous rather than a batch operation.

Since chromium losses in my process are negligible, the total degree of iron removal accrues to the benefit of the improved chromium:iron ratio, and since the chromium, aluminum, and magnesium oxides are relatively unaffected in the process, all reagents consumed are almost 100% efficient as regards iron removal.

The formula for chromite is usually accepted to be FeO.Cr<sub>2</sub>O<sub>3</sub>. The dot between the ferrous oxide component and the chromic oxide component indicates that there are two radicals present (a radical being a group of atoms which behave as an entity) which are somewhat loosely connected. FeO is usually soluble in common reagent acids without difficulty, but since chromite can be ground very fine and agitated for long periods in varying strengths of sulphuric acid without appreciable decomposition or without solution of appreciable quanti-

2

ties of iron, the FeO is evidently protected in chromite by the Cr<sub>2</sub>O<sub>3</sub> radical. The FeO also appears to be protected against reduction since intense heating of chromite in a reducing atmosphere renders it only slightly more magnetic and only slightly more susceptible to attack by sulphuric acid of any strength. On the other hand, the FeO does not appear to have as much protection against oxidation, since samples of chromite of 10 mesh size which have been wetted and subsequently dried slowly turn from shiny black to dull brown. Such accidentally air-oxidized chromite can be caused to become noticeably magnetic by heating to redness in a reducing atmosphere.

I have found that chromite ores of any grade and of any chromium:iron ratio can be thoroughly oxidized by roasting at approximately 700° C. with access of air and constant rabbling. The time required for thorough oxidation depends upon the accessibility of air, the efficiency of rabbling, and the maximum particle size. One-fourth inch material can be oxidized but I prefer to use minus 10 mesh chromite, since minus 10 mesh material gives me more rapid oxidation than coarser sizes, and less dusting than does finer sizes. With good air supply and good rabbling, on a thin bed, 30 minutes is sufficient time for oxidation, but in making tests with hand rabbling I prefer to use a three-hour oxidizing period when plotting variables other than length-of-oxidation period.

Since we start with FeO.Cr<sub>2</sub>O<sub>3</sub>, and oxidize at 700° C., I theorize the iron, after oxidation, must be in the form of Fe<sub>2</sub>O<sub>3</sub>. This conclusion is fortified by the fact that the oxidized product is nonmagnetic, is only very slightly attacked by sulphuric acid at any strength, and shows the slight increase in weight necessary to support such assumption. Since there are now two atoms of iron in the Fe radical, the formula for the oxidized chromite must be written Fe<sub>2</sub>O<sub>3</sub>.2Cr<sub>2</sub>O<sub>3</sub> as the chromium to iron proportions have not been changed. I prefer to show the new arrangement thusly,



The oxidation reaction formula is 4(FeO.Cr<sub>2</sub>O<sub>3</sub>) plus O<sub>2</sub> equals 2Fe<sub>2</sub>O<sub>3</sub>.4Cr<sub>2</sub>O<sub>3</sub>.

I have found that the iron in the oxidized product can be readily preferentially reduced by exposure to a reducing atmosphere such as one high in carbon monoxide or hydrogen at a temperature of approximately 1200° C. For laboratory tests, I prefer to mix the minus 10 mesh oxidized product with about 15% of its own weight of minus 10 mesh ordinary low-grade bituminous coal and reduce the charge for four hours at 1200–1260° C. in 30-gram fireclay crucibles. Using 15% coal means theoretically a great excess, but the 30-gram crucibles are only about six inches tall, consequently much CO<sub>2</sub> is expelled into the atmosphere. The efficiency of the reducing agent is dependent upon the opportunity it has for contact, therefore a long and narrow tube is much more efficient. I have obtained an equal amount of reduction with much less coal when working with a fire-clay tube three inches in inside diameter by eighteen inches long. I have also attained very satisfactory reduction in iron pipes, one inch by fifteen inches long and three inches diameter by fifteen inches long. The iron pipe does not enter into any reaction and does not corrode on the inside but soon crystallizes and breaks up from the outside because of the direct heat. In a large scale installation, reduction should be satisfactorily achieved in a rotary kiln and possibly in a roaster of the Fluo-Solids type for sizes fine enough for fluidizaiton. If a kiln were used, the reducing agent could not be gained from coal fed in with the ore, but would have to be fed as a gas into the discharge end of the kiln so as to travel counter-currently

to the chromite flow. An advantage of using a rotary kiln which could be realized also with certain other types of apparatus, lies in the fact that the hot exhaust gases from the kiln can be used as the source of heat for the prior oxidation reaction, and the hot oxidized chromite can be charged directly into the reducing apparatus without substantial loss of heat.

When coal or other hydrocarbons are used as the source of the reducing agent, and the reduction is performed in a tube-shaped vessel with at least one end having an aperture open so that there is no build-up in pressure, the iron in the chromite is preferentially reduced, in part, to an acid-soluble form. Such reduction takes place, to some extent, at all temperatures between 500 deg. C. and the fusing temperature of chromite (about 1500 deg. C.) but reductions at low temperature is slow and superficial. I prefer to use reducing temperatures of 1200-1260 deg. C. on minus 10 mesh material when using coal or other hydrocarbons, as the source of the reducing agent, in a relatively long, narrow vessel for a period of four hours total reduction time.

The formula for the reduction stage can be written—  
 $3\text{Fe}_2\text{O}_3 \cdot 6\text{Cr}_2\text{O}_3$  plus  $2\text{CO}$  equals  $\text{Fe}_3\text{O}_4$  plus  $3\text{FeO} \cdot 6\text{Cr}_2\text{O}_3$  plus  $2\text{CO}_2$ . I prefer to show the reactions in a manner that better demonstrates the reasons why re-arrangement of the chromite molecule is possible. In  $\text{FeO} \cdot \text{Cr}_2\text{O}_3$ , any reduction of the ferrous radical can only result in the formation of metallic Fe. To change the iron to a readily soluble form requires oxidation to  $\text{Fe}_3\text{O}_4$ . This cannot be done directly because direct oxidation results in the highest common state of oxidation,  $\text{Fe}_2\text{O}_3$ . When the iron is oxidized to  $\text{Fe}_2\text{O}_3$ , there must necessarily be two  $\text{Cr}_2\text{O}_3$  radicals to each one  $\text{Fe}_2\text{O}_3$  radical to make the number of atoms present of each be in balance. Instead of writing the formula as  $\text{Fe}_2\text{O}_3 \cdot 2\text{Cr}_2\text{O}_3$ , I prefer to show it as



Thus, while one chromium-bearing radical ordinarily protects its respective iron-bearing radical from attack, we now have a new molecular arrangement in which two chromium-bearing radicals are satisfied with sharing one iron-bearing radical. Then, when the iron-bearing radical is reduced to a lower state of oxidation, only half of the iron is retained as  $\text{FeO}$  to satisfy the newly-acquired requirements of the molecule for a one-iron radical:two-chromium radicals ratio. The entire set of equations may be written in balanced form as—

In oxidation



or to show the molecular arrangement



Then the reduction reaction



can be shown as



in which each  $\text{FeO}$  radical is sufficient to satisfy two  $\text{Cr}_2\text{O}_3$  radicals, the possibility of which is proved by the fact that the iron can be caused to go into a state of oxidation higher than the original  $\text{FeO}$ . I have found that it is possible, with the use of sufficient reducing agent, to cause more drastic re-arrangement on the same system by causing one  $\text{FeO}$  radical to satisfy more than two  $\text{Cr}_2\text{O}_3$  radicals, but when this is done, more drastic leaching procedures are necessary to extract all the available iron and recovery of chromite falls sharply.

From chromite ore reduced in the above manner, about one-half of the original iron content is readily soluble without further grinding, in dilute sulphuric acid or in

75

sulphurous acid (a solution of  $\text{SO}_2$  gas in water) while  $\text{Cr}_2\text{O}_3$  is attacked hardly at all, usually to the extent of less than one percent of the contained  $\text{Cr}_2\text{O}_3$ . If ferric sulphate is added to dilute sulphuric acid, no more iron is soluble than when dilute sulphuric acid alone is used, and the speed of iron-leaching is not increased. I take this as evidence that little of the iron has been reduced to metallic Fe, and the order of weight changes that take place during reduction further substantiate this conclusion. Since the reduced product is highly magnetic to a hand magnet, the resultant acid-soluble iron must be in the form of magnetite,  $\text{Fe}_3\text{O}_4$ .

In most chromite ores, at the end of the reduction step, it is found that ten or fifteen percent of the product is not as magnetic to a hand magnet as the balance of the product. This ten or fifteen percent fraction, which is less magnetic, proves by assay to be lower in both iron and chromium than the bulk of the product, and is slightly less magnetic because of the difference in composition and not because of lack of reduction. Also, the chromium:iron ratio is usually higher in this fraction than it is in the more highly magnetic portion, which helps to compensate for the fact that the iron in the less-magnetic fraction is more resistant to the subsequent leaching.

A sample of chromite ore of unknown origin was crushed to minus 10 mesh size, oxidized in air with hand-rabbling for three hours at 750 deg. C., mixed with 15% of its own weight of minus 10 mesh coal and reduced in an iron pipe three inches inside diameter by fifteen inches long which was plugged at one end and fitted with a 3 in. by 1 in. bell reducer on the other end. Reduction was at 1200 deg. C. in a butane-fired furnace for three hours. 100 grams of the reduced product was separated with a hand-magnet into 85 grams of highly magnetic grains and 15 grams of less magnetic grains. Assays made showed the following content of the respective fractions.

| Product              | Grams | Percent Cr | Percent Fe | Cr:Fe Ratio |
|----------------------|-------|------------|------------|-------------|
| Highly magnetic..... | 85    | 24.98      | 12.04      | 2.07:1      |
| Less magnetic.....   | 15    | 22.74      | 8.85       | 2.57:1      |

Subsequent leaching raised the ratio of the highly magnetic fraction to 3.16:1 and the leached product showed a loss in weight by leaching which was 3.9 times as great as the weight loss shown by the less magnetic product in which the ratio was raised only to 2.78:1.

Examination of the chromite particles at the end of the reduction step, under the microscope, reveals numerous straight brown lines which seemingly follow the exposed edges of parting planes, and a lesser number of small roughly circular brownish patches. After leaching of iron has been accomplished, examination of the particles under the microscope reveals that the brownish lines and patches have disappeared, leaving open crevices and craters. This migration of iron makes the subsequent leaching very rapid. I have found that chromite reduced in this manner and to this condition permits approximately one-half of its iron content to be extracted, at air temperature and at atmospheric pressure and without any further grinding to smaller size, by leaching with sulphuric acid of 33 1/3% strength (by volume) for one hour at atmospheric pressure and temperature, by leaching with sulphuric acid of 10% strength (by volume for reasonably longer periods, or by leaching with sulphurous acid (a solution of 6% by weight  $\text{SO}_2$  gas in water) for periods of from 20 minutes to 4 hours, depending upon the percentage of iron to be removed. Sulphurous acid of 3% strength requires a slightly longer leaching time to be employed than when 6%  $\text{SO}_2$  is used, if all the soluble iron is to be removed. Sulphurous acid of 6% strength dissolves as much or more iron in a shorter time than any strength of sulphuric acid solution when both are applied at air temperature.

Grinding of reduced chromite to a finer size, as to minus

100 mesh for example, and use of heated dilute sulphuric will hasten the leaching time to some degree, but I prefer to leach with sulphurous acid of 6% strength or nearly 6% strength at air temperature, without grinding finer than the size at which the chromite was reduced, for reasons of economy. With proper agitation during leaching, to insure constant contact of every particle with unsaturated leaching solution, the 20 minute leaching time is ample to put enough iron into solution to almost double the original chromium:iron ratio, and recovery of chromium in the unattacked residue is almost 100%, usually well over 99%, when leaching is done with sulphurous acid at air temperature.

When dilute sulphuric acid is used with moderate heating such as at 100 deg. C., but little more chromium is dissolved. At high concentrations of sulphuric acid applied at higher temperatures especially if done under pressure, greater amounts of chromium are lost as greater temperatures are applied and as pressure is increased, but in my improved process, such applications of heat and pressure, with resultant losses of chromium, are totally unnecessary. I prefer to use sulphurous acid, of 6% strength, or as nearly 6% as practical to supply, as the iron-leaching solvent, applying the solvent counter-currently to the flow of ore, so that the fresh solvent is applied on the oldest ore and the oldest solvent which has very little remaining  $\text{SO}_2$  is on the newest ore. By this means, almost 100% of the  $\text{SO}_2$  has been made available for the solution of iron and there is no necessity for the regeneration of the solvent. The used-up solvent can be discarded without noxious vapors or free acidity and with no wastage charge against it except for the water cost. The  $\text{SO}_2$  solution can be made by roasting pyrite (or other sulphides) and introducing the resultant  $\text{SO}_2$  gas into water by conventional means. If the used solvent were to be regenerated with  $\text{SO}_2$  gas, ferro sulphate and sulphuric acid would be formed by the well-known auto-oxidation process, and since these have been shown to be inferior to sulphurous acid for my purpose, interests of economy dictate the counter-current flow as described with discard of used lixiviant. Theoretically, with most chromite ores, roasting of 3 tons of pyrites will furnish enough  $\text{SO}_2$  to put 100 tons of chromite into the metallurgical grade class, as far as chromium:iron ratio is concerned.

The primary control over the degree of potential iron extraction desired lies in the quantity of reducing agent permitted to contact the chromite particles at reducing temperatures. Full utilization of available carbon monoxide requires higher temperatures than does full utilization of hydrogen. Very satisfactory final chromium:iron ratios can be attained on any chromite ores with a 99% plus chromite recovery if excessive reduction is avoided. Optimum reduction will vary with individual ores, but original chromium:iron ratios can be doubled in all instances without chromite losses exceeding 1%.

A 1-kilo batch of minus 10 mesh chromite of unknown derivation which had been concentrated by gravity to a product assaying 24.30% Cr and 12.05% Fe with a Cr:Fe ratio of 2.02:1 was roasted in an electric muffle furnace for 3 hours at approximately 700 deg. C. with free access of air but no appreciable draft. The charge was hand-rabbed during the roast. At the end of the oxidizing period, the charge was removed, cooled, and mixed with 20% of its own weight of minus 10 mesh low-grade bituminous coal. The mixture was poured into an iron pipe of one inch inside diameter and fourteen inches long. One end of the pipe was plugged and the other end was left open. This charge was heated from a cold start to approximately 1200 deg. C. in 30 minutes and held at approximately 1200 deg. C. for 2½ hours. At the end of the 3-hour reduction period the charge was quenched in water. Some coal not entirely consumed was washed out from the chromite. The chromite was all very magnetic to a hand magnet. Half of the reduced chromite product was ground to minus 100 mesh in a hand mortar and the

other half was left at minus 100 mesh. The following leach tests were made on the reduced products:

| 5  | Leach test | Mesh | Grams | Time     | Solvent                     | Temp., °C. | Agitation? |
|----|------------|------|-------|----------|-----------------------------|------------|------------|
| 1. |            | -100 | 10    | 3 hours  | 1:2 $\text{H}_2\text{SO}_4$ | 100        | Yes.       |
| 2. |            | -100 | 10    | 16 hours | 1:2 $\text{H}_2\text{SO}_4$ | 20         | Yes.       |
| 3. |            | -100 | 10    | 20 mins. | 6% $\text{SO}_2$ in water   | 20         | Yes.       |
| 10 | 4.         | -100 | 10    | 22 hours | 6% $\text{SO}_2$            | 20         | No.        |
|    | 5.         | -10  | 10    | 3 hours  | 1:2 $\text{H}_2\text{SO}_4$ | 100        | Yes.       |

The leached charges were filtered, dried, weighed and assayed for chromium and iron. Chromium recovery was calculated from chromium not found in filtrate.

#### RESULTS

| 20 | Leach Test | Weight | Percent Cr | Percent Fe | Cr:Fe Ratio | Percent Cr Recovery |
|----|------------|--------|------------|------------|-------------|---------------------|
| 1. |            | 9.26   | 26.27      | 6.43       | 4.09:1      | 99.37               |
| 2. |            | 9.35   | 26.34      | 6.49       | 4.06:1      | 99.42               |
| 3. |            | 9.47   | 26.16      | 7.49       | 3.49:1      | 99.58               |
| 25 | 4.         | 9.06   | 26.33      | 7.76       | 3.39:1      | 99.60               |
|    | 5.         | 9.38   | 26.37      | 7.20       | 3.66:1      | 99.52               |

10 grams of the minus 10 mesh material was then leached 4 hours with 6%  $\text{SO}_2$  in water solution at 20 deg. C. under 50 lbs./sq. in. pressure. 10 grams of minus 10 mesh material was leached 4 hours with 1:2  $\text{H}_2\text{SO}_4$  at 20 deg. C. under 50 lbs./sq. in. pressure. No agitation was applied to these tests.

#### RESULTS

| 40                               | Leach Test | Weight | Percent Cr | Percent Fe | Cr:Fe Ratio | Percent Cr Recovery |
|----------------------------------|------------|--------|------------|------------|-------------|---------------------|
| With $\text{SO}_2$               |            | 9.50   | 25.72      | 7.75       | 3.32:1      | 99.26               |
| With 1:2 $\text{H}_2\text{SO}_4$ |            | 9.55   | 25.65      | 7.53       | 3.41:1      | 99.25               |

45 Apparently these leaches were helped less by the pressure applied than they were hurt by the fact that no agitation could be applied.

1 kilo of minus 10 mesh chromite of unknown origin which had been concentrated by gravity to a product assaying 24.30% Cr, 12.05% Fe and 2.04%  $\text{SiO}_2$  with a Cr:Fe ratio of 2.02:1 was oxidized by roasting for 3 hours at a dull red heat on an iron plate on top of a butane-fired furnace with free access of air and constant hand-rabbling. At the end of the 3 hour oxidizing period, the charge was cooled and mixed with 20% of its own weight of minus 10 mesh low-grade bituminous coal. The chromite-coal mixture was poured into a tube of refractory fire-clay 3 inches in inside diameter by 14 inches long. One end of the tube was plugged, and the other end was partially plugged with refractory cement, leaving a 1 inch opening for gas escape and subsequent emptying. The charge in the tube was heated quickly—in less than 15 minutes—to 1260 deg. C. and held at that temperature four hours. Much of the coal was observed to burn before the chromite had become heated. At the end of the four hour reduction period, the charge was not quenched but was merely allowed to cool slowly in air. When the charge had cooled, it was split into two halves, one of which was left at minus 10 mesh, while the other half was ground to minus 100 mesh in a disc pulverizer. Numerous leaching tests were then made from which the leached residues were filtered, dried weighed and assayed, and from which the filtrates were assayed for chromium to establish the percentage of chromium recovery.

| Leach Test | Grams | Mesh | Solvent                                                                               | Time                 | Temp., °C. |
|------------|-------|------|---------------------------------------------------------------------------------------|----------------------|------------|
| a-----     | 10    | -10  | 1:2 H <sub>2</sub> SO <sub>4</sub>                                                    | 3 hours              | 100        |
| b-----     | 50    | -10  | 6% SO <sub>2</sub>                                                                    | 20 min.              | 20         |
| c-----     | 50    | -10  | 6% SO <sub>2</sub>                                                                    | 4 hours              | 20         |
| d-----     | 50    | -10  | 1:2 H <sub>2</sub> SO <sub>4</sub>                                                    | 20 min.              | 20         |
| e-----     | 50    | -10  | 1:2 H <sub>2</sub> SO <sub>4</sub>                                                    | 4 hours              | 20         |
| f-----     | 10    | -100 | 1:2 H <sub>2</sub> SO <sub>4</sub>                                                    | 3 hours              | 100        |
| g-----     | 50    | -100 | 6% SO <sub>2</sub>                                                                    | 20 min.              | 20         |
| h-----     | 50    | -100 | 6% SO <sub>2</sub>                                                                    | 4 hours              | 20         |
| i-----     | 50    | -100 | 1:2 H <sub>2</sub> SO <sub>4</sub>                                                    | 20 min.              | 20         |
| j-----     | 50    | -100 | 1:2 H <sub>2</sub> SO <sub>4</sub>                                                    | 4 hours              | 20         |
| k-----     | 50    | -100 | 6% SO <sub>2</sub>                                                                    | 5 min.               | 20         |
| l-----     | 50    | -100 | 1:2 H <sub>2</sub> SO <sub>4</sub>                                                    | 5 min.               | 20         |
| m-----     | 10    | -100 | 3% SO <sub>2</sub>                                                                    | 20 min.              | 20         |
| n-----     | 25    | -10  | 1:5 H <sub>2</sub> SO <sub>4</sub> plus 10 grams of Fe(SO <sub>4</sub> ) <sub>3</sub> | 4 hours              | 20         |
| o-----     | 25    | -10  | 6% SO <sub>2</sub> replaced with fresh SO <sub>2</sub> after 20 min.                  | 20 min. plus 20 min. | 20         |

## RESULTS

| Leach Test | Residue Weight | Percent Cr | Percent Fe | Cr:Fe Ratio | Percent Cr Recov. |
|------------|----------------|------------|------------|-------------|-------------------|
| a-----     | 9.39           | 26.13      | 7.47       | 3.50:1      | 99.37             |
| b-----     | 47.80          | 25.90      | 7.90       | 3.23:1      | 99.68             |
| c-----     | 47.68          | 25.93      | 7.72       | 3.26:1      | 99.83             |
| d-----     | 48.10          | 25.79      | 8.26       | 3.12:1      | 99.72             |
| e-----     | 47.96          | 25.79      | 8.14       | 3.17:1      | 99.71             |
| j-----     | 9.09           | 26.41      | 6.62       | 3.99:1      | 98.79             |
| g-----     | 47.31          | 26.10      | 7.35       | 3.55:1      | 99.82             |
| h-----     | 47.12          | 26.20      | 7.25       | 3.61:1      | 99.63             |
| i-----     | 47.36          | 26.10      | 7.47       | 3.49:1      | 99.69             |
| j-----     | 48.66          | 26.34      | 6.93       | 3.80:1      | 99.13             |
| k-----     | 48.46          | 25.65      | 8.63       | 2.97:1      | 99.86             |
| l-----     | 48.43          | 25.51      | 8.87       | 2.88:1      | 99.77             |
| m-----     | 9.68           | 25.75      | 8.51       | 3.03:1      | 99.62             |
| n-----     | 23.95          | 26.14      | 8.01       | 3.26:1      | 99.68             |
| o-----     | 23.86          | 26.07      | 8.24       | 3.16:1      | 99.65             |

These tests show a Cr:Fe ratio of better than 3:1 in all instances except "k" and "l" in which leaching time was cut to 5 minutes. They show, that while hot 1:2 H<sub>2</sub>SO<sub>4</sub> is the most effective solvent, cold leaching is as effective with SO<sub>2</sub> as 1:2 H<sub>2</sub>SO<sub>4</sub>; that ferric sulphate is of no benefit, and that, while minus 10 mesh material does not leach as fast as 100 mesh, leaching of 10 mesh is satisfactorily in leaching periods of as short as 20 minutes duration.

1 kilo of minus 10 mesh chromite of unknown origin which had been concentrated by gravity to a product assaying 22.87% Cr and 10.53% Fe with a chromium:iron ratio of 2.17:1, without prior oxidation was mixed with 20% of its own weight of minus 10 mesh low-grade bituminous coal and poured into a refractory fire-clay tube of 3 inches inside diameter by 14 inches long. One end was plugged and one end was partially plugged leaving a 1-inch circular opening. This charge was heated to 1200 deg. C. and reduced for four hours in a butane-fired furnace. The charge was then quenched in water, cleaned of unconsumed coal, and dried. 50 grams of the reduced chromite was leached for 20 minutes with 1:2 H<sub>2</sub>SO<sub>4</sub> at 100 deg. C. The leached charge was filtered, dried, weighed and assayed. The leached residue weighed 48.81 grams, assayed 24.94% Cr and 9.18% Fe which showed a Cr:Fe ratio of 2.72:1. The conclusion is that prior oxidation is necessary and probably the only reason that some change in ratio was effected here, was because of air-oxidation present in the old sample before treatment, and/or because of some oxidation taking place in the charge in the early stages of the intended reduction period.

A sample of chromite of unknown origin consisting of particles as large as  $\frac{1}{4}$  inch down to 10 mesh size was screened to eliminate all plus  $\frac{1}{4}$  inch and all minus 10 mesh. The resultant minus  $\frac{1}{4}$  inch, plus 10 mesh material which assayed 22.87% Cr and 10.53% Fe with a Cr:Fe ratio of 2.17:1 was given an oxidizing roast at 700-750 deg. C. for 3 hours, hand-rabbed, on an iron plate on top of the butane-fired furnace. At the end of the 3-hour oxidation period, the charge was cooled and mixed with 20% of its own weight in minus 10 mesh

coal. This mixture was poured into the 3-inch tube and reduced in the butane furnace for four hours at 1200 deg. C. At the end of the four hour reduction period, the charge was quenched in water, washed free of unconsumed coal and dried. The reduced chromite was split into two halves, one-half pulverized to minus 100 mesh in a disc pulverizer, and the other half was left at plus 10 mesh-minus  $\frac{1}{4}$  inch for leaching tests. All tests were performed in rolling bottles.

| Leach Test | Grams | Mesh                      | Solvent                                                                                         | Time    | Temperature, °C. |
|------------|-------|---------------------------|-------------------------------------------------------------------------------------------------|---------|------------------|
| a-----     | 25    | plus 10 - $\frac{1}{4}$ " | 6% SO <sub>2</sub>                                                                              | 20 min. | 20               |
| b-----     | 25    | plus 10 - $\frac{1}{4}$ " | 6% SO <sub>2</sub>                                                                              | 4 hours | 20               |
| c-----     | 25    | plus 10 - $\frac{1}{4}$ " | 1:2 H <sub>2</sub> SO <sub>4</sub>                                                              | 20 min. | 20               |
| d-----     | 25    | plus 10 - $\frac{1}{4}$ " | 1:2 H <sub>2</sub> SO <sub>4</sub>                                                              | 4 hours | 20               |
| e-----     | 25    | -100                      | 6% SO <sub>2</sub>                                                                              | 20 min. | 20               |
| f-----     | 25    | -100                      | 6% SO <sub>2</sub>                                                                              | 4 hours | 20               |
| g-----     | 25    | -100                      | 1:2 H <sub>2</sub> SO <sub>4</sub>                                                              | 20 min. | 20               |
| h-----     | 25    | -100                      | 1:2 H <sub>2</sub> SO <sub>4</sub>                                                              | 4 hours | 20               |
| i-----     | 25    | -100                      | 1:2 H <sub>2</sub> SO <sub>4</sub>                                                              | 4 hours | 20               |
| j-----     | 25    | -100                      | 1:5 H <sub>2</sub> SO <sub>4</sub> plus 10 gms. Fe <sub>2</sub> (SO <sub>4</sub> ) <sub>3</sub> | 4 hours | 20               |

| Leach Test | Weight of Residue | Percent Cr | Percent Fe | Cr:Fe Ratio |
|------------|-------------------|------------|------------|-------------|
| a-----     | 24.71             | 23.48      | 9.31       | 2.52:1      |
| b-----     | 24.41             | 23.91      | 8.84       | 2.70:1      |
| c-----     | 24.77             | 23.35      | 9.78       | 2.39:1      |
| d-----     | 24.50             | 23.64      | 9.05       | 2.61:1      |
| e-----     | 24.12             | 24.25      | 8.40       | 2.89:1      |
| f-----     | 24.14             | 24.26      | 8.46       | 2.87:1      |
| g-----     | 24.02             | 24.32      | 8.48       | 2.87:1      |
| h-----     | 23.97             | 24.72      | 8.30       | 2.98:1      |
| i-----     | 24.40             | 24.04      | 9.55       | 2.52:1      |
| j-----     | 23.90             | 24.79      | 8.54       | 2.90:1      |

Chromium was found in leach solutions in this series in trace amounts only. Although the altered ratios attained here are short of the desired 3:1, the results are indicative of the surprising amount of oxidation and reduction that can be made to occur at relatively coarse sizes.

A 5-kilo sample of lump chromite marked "Dr. Iten's High-Grade Specimens" was crushed to minus 10 mesh size. The sample assayed 40.56% Cr and 10.28% Fe showing a Cr:Fe ratio of 3.95:1. 1 kilo of the minus 10 mesh material was given an oxidizing roast for 3 hours at 750 deg. C. on an iron plate on top of a butane-fired furnace, with constant hand-rabbling. At the end of the 3-hour oxidation period, the charge was cooled and mixed with 16% of its own weight in minus 10 mesh low-grade coal. This mixture was poured into two 30-gram fire-clay crucibles which were covered with loose-fitting porcelain covers. The charges were reduced by heating to 1260 deg. C. for four hours in the butane-fired furnace. At the end of the reduction period, when the porcelain covers were removed, each cover was coated on its lower surface with a disc of elemental carbon foil, which demonstrated the waste of reducing agent that occurs in vessels of the dimensions of crucibles.

The charges from the two crucibles were quenched in water, combined, washed free from unconsumed coal and dried. The reduced product was then split into two halves, one half of which was pulverized to minus 100 mesh in a hand mortar while the other half was left at minus 10 mesh for leaching tests.

| Leach Test | Grams | Mesh | Solvent                            | Time    | Temp., °C. |
|------------|-------|------|------------------------------------|---------|------------|
| a-----     | 10    | -10  | 1:2 H <sub>2</sub> SO <sub>4</sub> | 30 min. | 100        |
| c-----     | 25    | -10  | 6% SO <sub>2</sub>                 | 20 min. | 20         |
| d-----     | 25    | -10  | 1:2 H <sub>2</sub> SO <sub>4</sub> | 20 min. | 20         |
| e-----     | 25    | -10  | 1:2 H <sub>2</sub> SO <sub>4</sub> | 4 hours | 20         |
| b-----     | 10    | -100 | 1:2 H <sub>2</sub> SO <sub>4</sub> | 30 min. | 100        |
| f-----     | 25    | -100 | 6% SO <sub>2</sub>                 | 20 min. | 20         |
| g-----     | 25    | -100 | 1:2 H <sub>2</sub> SO <sub>4</sub> | 20 min. | 20         |
| h-----     | 25    | -100 | 1:2 H <sub>2</sub> SO <sub>4</sub> | 4 hours | 20         |

## RESULTS

| Leached Test | Residue Weight | Percent Cr | Percent Fe | Cr:Fe Ratio | Percent Cr Recov. |
|--------------|----------------|------------|------------|-------------|-------------------|
| a-----       | 9.64           | 42.27      | 8.41       | 5.03:1      | 99.16             |
| c-----       | 24.55          | 41.79      | 9.09       | 4.60:1      | 99.34             |
| d-----       | 24.56          | 41.56      | 9.09       | 4.57:1      | 99.30             |
| e-----       | 24.35          | 42.06      | 8.62       | 4.88:1      | 99.33             |
| f-----       | 9.30           | 43.02      | 7.92       | 5.43:1      | 99.83             |
| j-----       | 24.10          | 42.34      | 8.29       | 5.11:1      | 99.13             |
| g-----       | 24.17          | 41.65      | 8.29       | 5.02:1      | 99.09             |
| h-----       | 23.00          | 42.61      | 8.04       | 5.30:1      | 98.47             |

This test was run more in a qualitative spirit than to determine exact quantitative results, and these results would be much better if the vessels used in the reducing step had been relatively longer and narrower than the short squat crucibles employed. Taking into consideration the erratics allowable in assaying, it is evident that sulphurous acid (a solution of 6%  $\text{SO}_2$  gas in water) is equal to or superior to much stronger concentrations of  $\text{H}_2\text{SO}_4$  when leaching is done at air temperature and leaching time is confined to the short times allowable in a continuous process.

A large sample of chromite ore, marked "Lumne Chromite" was crushed to minus 10 mesh size and concentrated by gravity to a concentrate assaying 28.34% Cr, 12.38% Fe and 2.40%  $\text{SiO}_2$ , showing a Cr:Fe ratio of 2.29:1. This minus 10 mesh concentrate was given an oxidizing roast for 3 hours at a dull red heat on an iron plate on top of the butane-fired furnace, with constant hand-rabbling. At the end of the 3-hour oxidation period, the charge was cooled and mixed with 16% of its own weight of minus 10 mesh low-grade coal. This mixture was poured into two 30-gram fire-clay crucibles and covered with loose-fitting porcelain covers. The two crucibles were placed in the butane-fired furnace and heated to 1260 deg. C. At the end of two hours, one crucible was removed and its charge quenched in water. The temperature was increased to 1370 deg. C. for the next two hours. At the end of the second two-hour period, the second crucible was removed and its charge quenched in water. The two charges were washed free of remaining unconsumed coal and then dried. Each of the two products was split into two halves, one half of which was ground to minus 100 mesh in a hand mortar while the other half was left at minus 10 mesh for leaching tests.

## LEACHING TESTS ON 2-HOUR REDUCTION TIME

| Leach Test | Grams | Mesh | Solvent                            | Leach Time hrs. |
|------------|-------|------|------------------------------------|-----------------|
| 1-----     | 25    | -10  | 1:2 $\text{H}_2\text{SO}_4$ -----  | 16              |
| 2-----     | 25    | -100 | 1:2 $\text{H}_2\text{SO}_4$ -----  | 16              |
| 3-----     | 25    | -10  | 1:10 $\text{H}_2\text{SO}_4$ ----- | 16              |
| 4-----     | 25    | -100 | 1:10 $\text{H}_2\text{SO}_4$ ----- | 16              |

## RESULTS OF LEACHING TESTS ON 2-HOUR REDUCTION TIME

| Leach Test | Residue Weight | Percent Cr | Percent Fe | Cr:Fe Ratio | Percent Cr Recov. |
|------------|----------------|------------|------------|-------------|-------------------|
| 1-----     | 24.66          | 28.93      | 11.11      | 2.60:1      | 99.73             |
| 2-----     | 24.51          | 29.26      | 11.08      | 2.64:1      | 99.69             |
| 3-----     | 24.50          | 29.26      | 11.14      | 2.63:1      | 99.71             |
| 4-----     | 24.29          | 29.46      | 11.31      | 2.60:1      | 99.72             |

## LEACHING TESTS ON 4-HOUR REDUCTION TIME

| Leach Test | Grams | Mesh | Solvent                            | Leach Time hrs. |
|------------|-------|------|------------------------------------|-----------------|
| 5-----     | 25    | -10  | 1:2 $\text{H}_2\text{SO}_4$ -----  | 16              |
| 6-----     | 25    | -100 | 1:2 $\text{H}_2\text{SO}_4$ -----  | 16              |
| 7-----     | 25    | -10  | 1:10 $\text{H}_2\text{SO}_4$ ----- | 16              |
| 8-----     | 25    | -100 | 1:10 $\text{H}_2\text{SO}_4$ ----- | 16              |

## RESULTS OF LEACHING TESTS ON 4-HOUR REDUCTION TIME

| Leach Test | Residue Weight | Percent Cr | Percent Fe | Cr:Fe Ratio | Percent Cr Recov. |
|------------|----------------|------------|------------|-------------|-------------------|
| 5-----     | 23.90          | 29.49      | 9.38       | 3.14:1      | 99.08             |
| 6-----     | 23.50          | 29.86      | 9.03       | 3.31:1      | 98.91             |
| 7-----     | 23.81          | 29.73      | 9.35       | 3.18:1      | 99.11             |
| 8-----     | 23.53          | 30.16      | 9.20       | 3.28:1      | 99.00             |

Apparently two hours' reduction time was not sufficient under existing conditions. 1:10 (by volume)  $\text{H}_2\text{SO}_4$  is as effective as 1:2  $\text{H}_2\text{SO}_4$  when leaching times of 16 hours are employed. Also iron extraction is almost as satisfactory at 10 mesh as it is at 100 mesh when a 16-hour leaching time is used.

A large sample of lump chromite ore marked "Silli Chromite" was crushed to minus 10 mesh and concentrated by gravity to a product assaying 28.54% Cr, 11.86% Fe and 2.26%  $\text{SiO}_2$ , showing a Cr:Fe ratio of 2.41:1. One kilo of this concentrate was given an oxidizing roast on an iron plate on top of the butane-fired furnace for 3 hours at a dull red heat, with constant hand-rabbling. At the end of the 3-hour oxidizing period, the charge was cooled and mixed with 16% of its own weight of low-grade coal. The mixture was poured into two 30-gram fire-clay crucibles and covered with loose-fitting porcelain covers. These were heated in the butane furnace to 1260 deg. C. At the end of two hours, one crucible was removed and its charge quenched in water. The temperature was increased to 1370 deg. C. for the next two hours. At the end of the second two-hour period, the second crucible was removed and its charge quenched in water. The two charges were washed free of remaining unconsumed coal and then dried. Each of the two products was split into two halves, one half of which was ground to minus 100 mesh in a hand mortar while the other half was left at minus 10 mesh for leaching tests.

## LEACHING TESTS ON 2-HOUR REDUCTION TIME

| Leach Test | Grams | Mesh | Solvent                            | Leach Time, hrs. |
|------------|-------|------|------------------------------------|------------------|
| 1-----     | 25    | -10  | 1:2 $\text{H}_2\text{SO}_4$ -----  | 16               |
| 2-----     | 25    | -100 | 1:2 $\text{H}_2\text{SO}_4$ -----  | 16               |
| 3-----     | 25    | -10  | 1:10 $\text{H}_2\text{SO}_4$ ----- | 16               |
| 4-----     | 25    | -100 | 1:10 $\text{H}_2\text{SO}_4$ ----- | 16               |

## RESULTS OF LEACHING TESTS ON 2-HOUR REDUCTION TIME

| Leach Test | Residue Weight | Percent Cr | Percent Fe | Cr:Fe Ratio | Percent Cr Recov. |
|------------|----------------|------------|------------|-------------|-------------------|
| 1-----     | 24.50          | 29.26      | 10.24      | 2.86:1      | 99.81             |
| 2-----     | 24.76          | 29.36      | 10.44      | 2.81:1      | 99.83             |
| 3-----     | 24.41          | 29.49      | 10.39      | 2.84:1      | 99.83             |
| 4-----     | 24.20          | 29.76      | 10.59      | 2.81:1      | 99.84             |

## LEACHING TESTS ON 4-HOUR REDUCTION TIME

| Leach Test | Grams | Mesh | Solvent                            | Leach Time hrs. |
|------------|-------|------|------------------------------------|-----------------|
| 5-----     | 25    | -10  | 1:2 $\text{H}_2\text{SO}_4$ -----  | 16              |
| 6-----     | 25    | -100 | 1:2 $\text{H}_2\text{SO}_4$ -----  | 16              |
| 7-----     | 25    | -10  | 1:10 $\text{H}_2\text{SO}_4$ ----- | 16              |
| 8-----     | 25    | -100 | 1:10 $\text{H}_2\text{SO}_4$ ----- | 16              |

## RESULTS OF LEACHING TESTS ON 4-HOUR REDUCTION TIME

| Leach Test | Residue Weight | Percent Cr | Percent Fe | Cr:Fe Ratio | Percent Cr Recov. |
|------------|----------------|------------|------------|-------------|-------------------|
| 5-----     | 23.81          | 29.03      | 9.43       | 3.08:1      | 95.68             |
| 6-----     | 23.71          | 30.06      | 9.06       | 3.32:1      | 98.83             |
| 7-----     | 23.80          | 29.56      | 10.62      | 2.78:1      | 97.62             |
| 8-----     | 23.54          | 30.23      | 9.17       | 3.30:1      | 99.01             |

Reduction time of two hours, under existing conditions was not enough. Four hour reduction time was sufficient, but evidently higher temperature employed (1370 deg. C.) during the latter two hours led to greater chromium losses and somewhat lesser iron solubility. I have observed partial fusion of chromite at temperatures of only 30 or 40 degrees above the peak reached here. A temperature of 1260 deg. C. should be the upper working limit.

What is claimed is:

1. A process of upgrading chromite ore having an initial Cr:Fe ratio of less than 3:1 to a metallurgical grade chromite ore having a final Cr:Fe ratio of more than 3:1 wherein FeO and Cr<sub>2</sub>O<sub>3</sub> are molecularly bonded in both the initial ore and in the metallurgical grade ore comprising the steps of comminuting the ore, heating the comminuted ore at a preferred temperature range of about 700° to 750° centigrade under oxidizing conditions while controlling the degree of comminution, the heating temperature and the oxidizing conditions so as to oxidize at least a portion of the FeO.Cr<sub>2</sub>O<sub>3</sub> therein to

Fe<sub>2</sub>O<sub>3</sub>.2Cr<sub>2</sub>O<sub>3</sub>, reducing at least a portion of said Fe<sub>2</sub>O<sub>3</sub>.2Cr<sub>2</sub>O<sub>3</sub> at a temperature range of about 1200° to 1370° centigrade to FeO.2Cr<sub>2</sub>O<sub>3</sub> and uncombined Fe<sub>3</sub>O<sub>4</sub> while leaving the Cr<sub>2</sub>O<sub>3</sub> substantially unchanged, and extracting said uncombined Fe<sub>3</sub>O<sub>4</sub> with a chemical reagent reactive therewith, whereby the ratio of Cr to Fe is increased.

5 2. A process as set forth in claim 1, wherein said reduction is conducted at a preferred temperature range of about 1200 to 1260 degrees centigrade.

10 3. A process as set forth in claim 2, wherein said reduction is conducted in an atmosphere of carbon monoxide.

15 References Cited in the file of this patent

UNITED STATES PATENTS

|           |              |       |               |
|-----------|--------------|-------|---------------|
| 153,573   | Kidwell      | ----- | July 28, 1874 |
| 1,196,049 | Rauschenplat | ----- | Aug. 29, 1916 |
| 1,360,666 | Mills        | ----- | Nov. 30, 1920 |
| 1,403,237 | Eustis       | ----- | Jan. 10, 1922 |
| 2,123,240 | Hammarberg   | ----- | July 12, 1938 |